

1

3,499,839  
AMINE-STABILIZED IODINE-CONTAINING  
LUBRICANTS

Julius Boehm, Cleveland, Ohio, assignor to The Standard  
Oil Company, Cleveland, Ohio, a corporation of Ohio  
No Drawing. Filed June 27, 1967, Ser. No. 649,137  
Int. Cl. C10m 3/02, 3/26, 1/40  
U.S. Cl. 252—33.4

1 Claim

### ABSTRACT OF THE DISCLOSURE

A lubricating oil having enhanced lubricating properties comprising a hydrocarbon lubricating oil, elemental iodine, a petroleum sulfonate, chlorinated wax and an amine.

This invention relates to addition of an amine to iodine-containing lubricants for enhancing lubricating properties of the lubricants and for imparting performance and storage stability thereto.

The invention disclosed herein relates to the field of iodine-containing lubricant compositions. It has been recently discovered that a small quantity of iodine in a carrier medium will act as an exceptionally effective oiliness agent to reduce friction occurring between moving surfaces. The iodine is particularly effective in improving lubricity of metal surfaces such as chrome, nickel, titanium, tungsten, and their alloys.

Roberts et al. Patent 3,228,880 discloses a lubricant comprising a charge transfer complex of iodine and an aromatic hydrocarbon which is especially useful on lubricating contacting surfaces at least one of which is 50 percent or more by weight titanium. Furey Patent 3,184,409 relates to (1) the use of elemental iodine in lubricating oil compositions for reducing friction between moving surfaces under boundary lubrication conditions and (2) elimination of iodine staining by incorporating certain compounds for that purpose. Furey et al. Patent 3,184,413 relates to polymeric lubricant compositions containing iodine for improving antifriction, antiwear and extreme pressure properties. Bell et al. Patent 3,220,949 relates to the discovery that inclusion of ashless nitrogen-containing oil-soluble derivatives of alkenyl succinic anhydrides in iodine-containing lubricants effectively reduces the corrosive effects of the iodine on metallic surfaces.

Although the iodine-containing lubricants provide such a dramatic improvement in lubrication of chrome, nickel, tungsten and titanium metals and their alloys over lubricants not containing any iodine, at present, there are no commercially available iodine-containing lubricants on the market. The reason for commercial non-availability of the iodine-containing lubricants resides in the fact that iodine-containing lubricants lack sufficient performance and storage stability. Upon standing for a short duration, effectiveness of the iodine as an oiliness agent in a lubricant is lost with a consequent loss of lubricity.

It has now been discovered that an amine in an iodine-containing lubricant will provide enhancement of lubricating properties of said lubricant as well as performance and storage stability so necessary for commercial exploitation of these lubricants.

Lubricants of the present invention comprise a hydrocarbon oil by lubricating viscosity, iodine, a sulfonate, chlorinated wax, and other additives as, for example, oxidation inhibitors such as phenothiazine or phenyl- $\alpha$ -naphthylamine and generally phenols, naphthols, sulfides and phosphides; detergent additives such as the barium salt of isononyl phenol sulfide and generally salts of phenols, of carboxylic acids, of sulfonic acids, and of alkyl phosphoric acids; pour-point depressants such as copolymers of vinyl acetate with fumaric acid esters of

2

coconut oil alcohols and more broadly, alkyl naphthenates, polymers of long-chain acrylates, and multivalent metal soaps of various fatty acids; viscosity index improvers such as polymethacrylates; foam depressants such as siloxane derivatives; rust preventives such as fatty acids and their oil-soluble alkaline earth salts, and multivalent metal salts of petroleum sulfonic acids; etc.

Suitable mineral or hydrocarbon oils of lubricating viscosity are the hydrocarbon lubricants obtained from petroleum. These products normally have viscosity in the range of 50 to 2000 Saybolt Universal Seconds at 100° F. The preferred hydrocarbon oils are those boiling above 300° F. and especially preferred are those boiling above 500° F. at atmospheric pressure. Solid products such as 15 paraffin wax, semi-solid products such as petrolatum and greases, or relatively non-viscous products like kerosine, gas oil or fuel oil are contemplated as suitable mediums for the additives. Additionally, various synthetic lubricating oils made from esters, polysiloxanes, carbonates, formals, polyglycols, and the like may likewise be utilized as mediums. The term "hydrocarbon oil of lubricating viscosity" is not intended to be limited to any specific application but may include cutting oils, metal working oils, pneumatic equipment oils, spindle oils, gear oils, 25 motor oils, etc.

Iodine can be utilized in its elemental state, as a charge transfer complex with a hydrocarbon, in a compound state, or as a component of a polymeric lubricating oil additive. The amount of iodine may range from 0.001 30 weight percent and up, but is generally in the range of about 0.001 to 10 weight percent and preferably in the range of about 0.01 to 0.5 weight percent.

Oil-soluble emulsifiers, such as sulfonates, which are derivatives of organic sulfonic acids, are used in amounts 35 of about 1 to 25 weight percent, and preferably in amounts of about 1 to 10 weight percent. The sulfonates function to solubilize the iodine as well as the amine. Examples of other emulsifiers are the alkali-metal salts of carboxylic and sulfonic acids, monoesters of polyhydric alcohols, ether alcohols, and the various polyoxyethylene derivatives of fatty acids.

Chlorinated wax and, generally, organic chlorine and sulfur compounds are used as extreme pressure additives. Chlorinated wax is used in an amount of about 1 to 25 weight percent and preferably in the amount of about 1 to 10 weight percent.

For more information on the various additives and applications of the lubricants containing such additives, reference is here made to the above-mentioned prior art patents, and the Kirk-Othmer Encyclopedia of Chemical Technology.

As was already pointed out, the present invention relates to the discovery that addition of an amine to an iodine-containing lubricating composition will impart thereto performance and storage stability and will enhance lubricating properties of the lubricant. Amines are added in an amount of about 0.001 to 10 weight percent and preferably in the amount of about 0.01 to 0.5 weight percent.

### Preparation of a lubricating composition

A typical lubricating composition was prepared by adding to a glass beaker 89.5 grams of oil having the following specification:

|                                 |       |
|---------------------------------|-------|
| 65 Gravity, °API                | 27.9  |
| Pour point, °F.                 | 20    |
| Flash point, °F.                | 35.5  |
| Color (ASTM test D-1500)        | L 2   |
| Viscosity, SSU/210° F., seconds | 38.87 |
| Viscosity, SSU/100° F., seconds | 100.0 |
| Viscosity index                 | 74    |
| Sulfur, weight percent          | 0.32  |

## Atmospheric distillation, ° F.:

|     |     |
|-----|-----|
| IBP | 601 |
| 2%  | 624 |
| 5%  | 659 |
| 10% | 669 |
| 20% | 680 |
| 30% | 694 |
| 40% | 712 |
| 50% | 722 |
| 60% | 740 |
| 70% | 759 |
| 80% | 781 |
| 90% | 810 |
| 95% | 832 |
| 98% | 858 |
|     | 15  |

The following ingredients were then added to the oil: 5 grams of a high molecular weight petroleum sulfonate; 5 grams of chlorinated wax; and 0.25 gram of elemental iodine.

The high molecular weight petroleum sulfonate had the following specifications:

|                             |          |
|-----------------------------|----------|
| Molecular weight            | 457      |
| Sulfonates                  | percent  |
| Mineral oil                 | do       |
| Inorganic salt              | do       |
| Water                       | do       |
| Specific gravity at 60° F.  | 1.02     |
| Weight per gallon at 60° F. | 8.50     |
| Furol viscosity at 210° F.  | 100      |
| Flash point                 | ° F. 380 |

The chlorinated wax had a viscosity of 165 SUS at 210° F. and contained 41 to 42 weight percent chlorine.

The contents of the beaker were heated to about 150° F. with constant stirring. After the iodine dissolved in the solution, heat was removed and 0.25 gram of triethanolamine was added with mixing.

To avoid formation of sludge, the sulfonate should be added before iodine, since the sulfonate acts to solubilize the iodine. The lower molecular weight amines are oil-insoluble and for that reason, should be added when a solubilizing agent, the sulfonate, is already in the solution. As one can surmize, the sulfonate acts as a dispersing and solubilizing agent for iodine as well as for the lower molecular weight amines. The higher molecular weight amines are oil-soluble, in which case, the sulfonate functions to solubilize only the iodine. Addition of more iodine and/or amine will require more sulfonate.

standard Falex testing machine using stainless steel V-blocks and brass test pins.

Table I shows results of Falex EP test of oils containing iodine on stainless steel test pins. In Table I, and subsequent tables, the acronym TEA represents triethanolamine; (W) indicates welding of the test piece at the particular load and termination of the test; and (S) indicates shearing of the shear pin, meaning that the load carrying capacity of the lubricating composition is higher than the recorded value. The load limit of the Falex machine is 4500 pounds, and in instances where this load was achieved, the test was terminated although the actual load capacity of the lubricant may have been above this figure.

TABLE I

| Blend | Blending date | Testing date | Weight percent iodine | Weight percent TEA | Load carrying capacity in pounds |
|-------|---------------|--------------|-----------------------|--------------------|----------------------------------|
| 1     | 9-2-66        | 9-2-66       | 0.1                   | -----              | 750 (W)                          |
| 1     | 9-2-66        | 9-5-66       | 0.1                   | -----              | 250 (W)                          |
| 2     | 9-6-66        | 9-6-66       | 0.1                   | 0.25               | 3,200 (S)                        |
| 2     | 9-6-66        | 11-14-66     | 0.1                   | 0.25               | 3,150 (S)                        |
| 3     | 9-9-66        | 9-9-66       | 0.25                  | -----              | 2,500 (W)                        |
| 3     | 9-9-66        | 9-20-66      | 0.25                  | -----              | 500 (W)                          |
| 3     | 10-5-66       | 10-6-66      | 0.25                  | 0.25               | 3,750 (S)                        |
| 4     | 9-9-66        | 9-9-66       | 0.25                  | 0.25               | 4,500                            |
| 4     | 9-9-66        | 11-14-66     | 0.25                  | 0.25               | 4,500                            |

Table I shows that Blend 1, without any triethanolamine, lost substantially all of its load carrying capacity in three days. Blend 2, containing 0.25 weight percent triethanolamine, retained its load carrying capacity even after standing for over two months. Blend 3 showed a load carrying capacity of 2500 pounds when tested on the day of blending, but lost substantially all of its load carrying capacity in ten days. Upon addition of 0.25 weight percent of triethanolamine on Oct. 5, 1966, to Blend 3, which was prepared on Sept. 6, 1966, its load carrying capacity was synergistically restored to 3750 pounds, which is 1250 pounds above its original load carrying capacity. Blend 4 shows that with 0.25 weight percent of iodine and 0.25 weight percent triethanolamine, the load carrying capacity exceeds 4500 pounds, and this value was retained even after two months. In general, the results in Table I show that amine dramatically improves storage stability and enhances performance of lubricating compositions containing iodine.

Another set of tests was conducted wherein the storage periods were further extended. The results are tabulated in Table II below.

TABLE II

|                 |           |           |           |           |           |           |
|-----------------|-----------|-----------|-----------|-----------|-----------|-----------|
| Oil             | 89.9      | 89.65     | 89.9      | 89.65     | 89.75     | 89.5      |
| Sulfonate       | 5.0       | 5.0       | 5.0       | 5.0       | 5.0       | 5.0       |
| Chlorinated wax | 5.0       | 5.0       | 5.0       | 5.0       | 5.0       | 5.0       |
| Iodine          | 0.1       | 0.1       | 0.1       | 0.1       | 0.25      | 0.25      |
| TEA             | 0.25      | -----     | 0.25      | -----     | 0.25      | 0.25      |
| Falex:          |           |           |           |           |           |           |
| Fresh           | 2,500 (W) | 3,500 (S) | 2,750 (W) | 3,750 (S) | 4,500     | 4,250 (S) |
| 2 weeks         | 750 (W)   | 1,000 (W) | -----     | 3,000 (W) | -----     | 4,500     |
| 4 weeks         | <250 (W)  | 3,250 (S) | 500 (W)   | 3,250 (S) | 1,750 (W) | 4,250 (S) |
| 8 weeks         |           | 3,250 (S) |           | 3,500 (S) | 1,000 (W) | 4,000 (S) |
| 12 weeks        |           |           |           |           | 500 (W)   | 4,250 (S) |

A preliminary test was conducted to determine effectiveness of triethanolamine in iodine lubricants with respect to performance and storage stability.

A number of lubricating compositions were prepared in accordance with above-described procedure, with the exception that amount of iodine and the amine was varied, as indicated in Table I below. The effectiveness of the particular lubricating composition was determined on a

Results in Table II confirm results obtained in previous tests. Especially significant is the last column which shows that the lubricating composition comprising 0.25 weight percent of iodine and 0.25 weight percent triethanolamine retained its load carrying capacity even after twelve weeks.

Table III shows the effect of varying amount of certain additives on load carrying capacity of the lubricating compositions.

TABLE III

|                 |       |       |       |       |       |       |       |       |       |       |       |       |       |       |       |       |
|-----------------|-------|-------|-------|-------|-------|-------|-------|-------|-------|-------|-------|-------|-------|-------|-------|-------|
| Oil             | 89.5  | 89.65 | 89.74 | 89.65 | 89.4  | 89.8  | 89.89 | 89.74 | 89.98 | 79.65 | 79.5  | 79.75 | 44.75 | 34.75 | 39.75 | 89.70 |
| Sulfonate       | 5.0   | 5.0   | 5.0   | 5.0   | 5.0   | 5.0   | 5.0   | 5.0   | 5.0   | 15.0  | 15.0  | 15.0  | 50.0  | 50.0  | 50.0  | 5.5   |
| Chlorinated wax | 5.0   | 5.0   | 5.0   | 5.0   | 5.0   | 5.0   | 5.0   | 5.0   | 5.0   | ----- | ----- | ----- | ----- | ----- | ----- | ----- |
| Iodine          | 0.25  | 0.25  | 0.25  | 0.1   | 0.1   | 0.1   | 0.1   | 0.01  | 0.01  | 0.25  | 0.25  | 0.25  | 0.25  | 0.25  | 0.25  | 0.25  |
| TEA             | 0.25  | 0.10  | 0.01  | 0.25  | 0.5   | 0.1   | 0.01  | 0.25  | 0.01  | 0.10  | 0.25  | ----- | 10.0  | 5.0   | 0.25  | ----- |
| Falex:          | (S)   | (S)   | (S)   | (S)   | (S)   | (S)   | (S)   | (S)   | (S)   | (W)   | (W)   | (S)   | (W)   | (W)   | (S)   | (S)   |
| Fresh           | 3,750 | 4,000 | 3,750 | 3,500 | 3,000 | 3,000 | 2,500 | 1,000 | 1,000 | 250   | 3,500 | 250   | 250   | 1,750 | 2,500 | <250  |
| 2 weeks         | 4,000 | 3,500 | 3,250 | 3,750 | 3,000 | 2,500 | 2,000 | 750   | 500   | 2,250 | 250   | 250   | 1,500 | 2,000 | ----- | ----- |
| 4 weeks         | 4,000 | 3,250 | 2,500 | 3,250 | 2,750 | 2,750 | 1,750 | 750   | 500   | 1,000 | ----- | 1,500 | 2,250 | 1,500 | 2,000 | ----- |

Table III indicates that best results are obtained with lubricating compositions comprising a sulfonate, chlorinated wax, and iodine and triethanolamine in an amount of 0.1 to 0.25 weight percent.

To determine effectiveness of triethanolamine on iodine-containing lubricants wherein iodine was in a form of iodine compounds, two lubricant blends were prepared using Mallinckrodt samples #2 and #15. The Mallinckrodt sample #2 was either an aliphatic or heterocyclic compound in which iodine was non-aromatic. Mallinckrodt sample #15 contained aromatic iodine. In sample #2, iodine content was in the range of 50 to 60 weight percent, while in sample #15, it was 60 to 85 weight percent. This constitutes all available pertinent information on these samples. The composition of these samples is regarded proprietary with the manufacturer.

The above lubricating compositions using iodine compounds were tested on the Falex machine with the following results.

TABLE IV

|                  |         |           |         |           |
|------------------|---------|-----------|---------|-----------|
| Oil              | 99.00   | 98.75     | 99.00   | 98.75     |
| Mallinckrodt #2  |         |           | 1.00    | 1.00      |
| Mallinckrodt #15 | 1.00    | 1.00      |         |           |
| TEA              |         | 0.25      |         | 0.25      |
| Sulfonate        |         | 5.00      |         | 5.00      |
| Falex:           |         |           |         |           |
| Fresh            | 250 (W) | 1,500 (W) | 250 (W) | 1,250 (W) |
| 2 weeks          |         | 1,750 (W) |         | 1,750 (W) |
| 4 weeks          |         | 1,750 (W) |         | 1,750 (W) |

A number of other amines have been found to impart desirable properties to the iodine-containing lubricants. Table V lists some of these amines and results of the Falex tests conducted on lubricating oil samples having the indicated composition.

TABLE V

|                     |       |       |       |       |       |       |       |       |       |       |       |
|---------------------|-------|-------|-------|-------|-------|-------|-------|-------|-------|-------|-------|
| Oil                 | 87.25 | 87.25 | 87.25 | 87.25 | 87.25 | 87.25 | 87.25 | 87.25 | 87.25 | 87.25 | 87.2  |
| Sulfonate           | 7.50  | 7.50  | 7.50  | 7.50  | 7.50  | 7.50  | 7.50  | 7.50  | 7.50  | 7.50  | 7.50  |
| Chlorinated Wax     | 5.00  | 5.00  | 5.00  | 5.00  | 5.00  | 5.00  | 5.00  | 5.00  | 5.00  | 5.00  | 5.00  |
| Iodine              | 0.25  | 0.25  | 0.25  | 0.25  | 0.25  | 0.25  | 0.25  | 0.25  | 0.25  | 0.25  | 0.25  |
| Triethanolamine     |       |       | 0.25  |       |       |       |       |       |       |       |       |
| Triisopropanolamine |       |       |       | 0.25  |       |       |       |       |       |       |       |
| Tri-n-butylamine    |       |       |       |       | 0.25  |       |       |       |       |       |       |
| Triethylamine       |       |       |       |       |       | 0.25  |       |       |       |       |       |
| Diethylamine        |       |       |       |       |       |       | 0.25  |       |       |       |       |
| Sec-butylamine      |       |       |       |       |       |       |       | 0.25  |       |       |       |
| n-Butylamine        |       |       |       |       |       |       |       |       | 0.25  |       |       |
| Aniline             |       |       |       |       |       |       |       |       |       | 0.25  |       |
| Diphenylamine       |       |       |       |       |       |       |       |       |       |       | 0.25  |
| N-ethylaniline      |       |       |       |       |       |       |       |       |       |       | 0.25  |
| Falex:              |       |       |       |       |       |       |       |       |       |       |       |
| Fresh               | 4,000 | 4,500 | 4,000 | 2,500 | 4,250 | 3,000 | 3,250 | 3,500 | 3,500 | 3,750 | 4,000 |
| 2 weeks             | 2,750 | 4,250 | 3,000 | 2,500 | 3,500 | 2,000 | 2,750 | 2,000 | 3,000 | 3,000 | 3,500 |
| 4 weeks             | 1,000 | 4,250 | 3,000 | 2,750 | 3,250 | 2,250 | 2,500 | 2,000 | 2,750 | 3,250 | 3,500 |

Examples of amines useful in the present invention for enhancing lubricating properties of the iodine-containing lubricants, and for imparting performance and storage stability thereto, are the following: methylamine, dimethylamine, trimethylamine, chlorine, ethylamine, diethylamine, triethylamine, n-propylamine, isopropylamine, aminomethylpropanol, monoisopropanolamine, diisopropanolamine, triisopropanolamine, butylamine, monoallylamine, amylamine, diamylamine, triamylamine, hexylamine, heptylamine, monoethanolamine, diethylethanolamine, triethanolamine, ethyl monoethanolamine, aminoethyl ethanolamine, aminoethylpropanol, benzylidimethylamine, ethylene diamine, diethylenetriamine, triethylene tetramine, tetraethylene pentamine, guanidine, diphenylguanidine, triphenylguanidine, diorthotolyguanidine, hexamethylenetetramine, aniline, formaldehyde-aniline condensation products, dimethylaniline, ethyl aniline,  $\beta$ -phenylethylamine, diethylaniline, ethylidene aniline, ethylbenzylaniline, cyclohexylamine, dicyclohexylamine, cyclopropylamine, (cyclohexylmethyl) amine, diphenylamine, o-phenylaniline, o-aminophenol, m-aminophenol, p-aminophenol, xylidine, diethyl-o-toluidine, o-phenylenediamine, p-phenylenediamine, m-phenylenediamine, p-diaminodiphenyl, m-toluidine, p-toluidine, N-ethyl-o-toluidine, N-ethyl-m-toluidine, N-ethyl-m-toluidine, methyl diethyl aminoben-

zene, diaminotoluene, methylene aniline, methylene di-aniline, p-aminoazobenzene, o-aminoazotoluene, diethylenediamine, amphetamine,  $\alpha$ -naphthylamine,  $\beta$ -naphthylamine, phenyl- $\alpha$ -naphthylamine, 1-cyclopentyl-2-amino-propane, bis(1-ethyl-3-methylpentyl)amine, diphenylamine, triphenylamine, octylamine, dodecylamine, tetradecylamine, hexadecylamine, octadecylamine, docosylamine, coco amine, tallow amine, hydrogenated-tallow amine, cottonseed amine, didodecylamine, ditetradecylamine, dihexadecylamine, dioctadecylamine, dicoco amine, dihydrogenated-tallow amine, di(eicosyl-docosyl)amine, trioctylamine, tridodecylamine, tricoco amine, isoctyldi-coco amine, trihydrogenated-tallow amine, N-methyl dihydrogenated-tallow amine, N,N-dimethyldecylamine, N,N-dimethyltetradecylamine, N,N-dimethylhexadecylamine, N,N-dimethyloctadecylamine, N,N-dimethylcoco amine, N,N-dimethyl(octadecenyl-octadecadienyl) amine, N,N-dimethyl hydrogenated-tallow amine, N-octadecenyltrimethylenediamine, N-coco trimethylenediamine, N-tallow trimethylenediamine, N-(octadecenyl-octadecadienyl)trimethylenediamine, 2-amino-1-butanol, 2-amino-2-methyl-1-propanol, polymeric amines such as polyethylamine, polyallylamine, etc.

The above group of compounds represents an attempt to list presently commercially available compounds useful in the instant invention. It is, however, intended to cover other related compounds, whether commercialized or not.

The useful compounds are classified into primary, secondary, and tertiary amines; and aliphatic amines from about 1 to about 36 carbon atoms, aromatic amines from about 6 to about 24 carbon atoms, alicyclic amines from about 3 to about 12 carbon atoms wherein the ring or

rings contain only carbon atoms, and polymeric amines. Preferably, the amines are classifiable into alkylamines from about 1 to about 15 carbon atoms, alkanolamines from about 2 to about 12 carbon atoms, and aromatic amines from about 6 to about 18 carbon atoms. Aromatic-aliphatic amines are to be considered as aromatic amines.

Although a gamut of amine compounds have been disclosed as being useful in the iodine-containing lubricants, it is intended to exclude related compounds such as ammonia, pyridine, picolines, quinolines, isoquinoline, quinaldine, indole, acridine, acridone, carbazoles, piperazines and the like.

It is intended to limit the present invention only to iodine-containing lubricants. Amount of an amine to be added to achieve storage and performance stability can be experimentally ascertained by a man ordinarily skilled in the art. Amount of iodine to be added is well documented in the herein noted prior art patents. Type and amounts of other additives for lubricants can be ascertained from prior art and will be dictated by requirements of a particular lubricant desired.

While the above invention has been described with a certain degree of particularity, it is realized that various additional modifications and adaptations can be made

within the spirit and scope of the invention as hereinafter claimed.

I claim:

1. In a lubricant comprising a major proportion of hydrocarbon oil of lubricating viscosity, elemental iodine in a friction-reducing amount, a high molecular weight petroleum sulfonate in an amount of about 1 to 10 weight percent chlorinated wax in an amount of about 1 to 10 weight percent, and an amine in an amount of about 0.01 to 0.5 weight percent, said amine is selected from the group consisting of

- (a) alkylamines from about 5 to about 15 carbon atoms,
- (b) alkanolamines from about 2 to about 12 carbon atoms, and
- (c) aromatic amines from about 6 to about 18 carbon atoms.

#### References Cited

#### UNITED STATES PATENTS

|             |         |                      |            |
|-------------|---------|----------------------|------------|
| 2,268,608   | 1/1942  | McNulty et al. ___   | 252—51.5 X |
| 3,184,409   | 1/1965  | Furey _____          | 252—58 X   |
| 5 3,220,949 | 11/1965 | Bell et al. _____    | 252—51.5   |
| 3,228,880   | 1/1966  | Roberts et al. _____ | 252—51     |
| 2,696,473   | 12/1954 | Sokol _____          | 252—51 X   |

DANIEL E. WYMAN, Primary Examiner

W. CANNON, Assistant Examiner

U.S. Cl. X.R.

252—49, 58

15

UNITED STATES PATENT OFFICE  
CERTIFICATE OF CORRECTION

Patent No. 3,499,839 Dated March 10, 1970

Inventor(s) Julius Boehm

It is certified that error appears in the above-identified patent and that said Letters Patent are hereby corrected as shown below:

Signed and sealed this 3rd day of August 1971.

(SEAL)  
Attest:

EDWARD M. FLETCHER, JR.  
Attesting Officer

WILLIAM E. SCHUYLER, JR.  
Commissioner of Patents